



US008733423B1

(12) **United States Patent**  
**Bornemann et al.**

(10) **Patent No.:** **US 8,733,423 B1**  
(45) **Date of Patent:** **May 27, 2014**

(54) **METAL ALLOY INJECTION MOLDING PROTRUSIONS**

(71) Applicant: **Microsoft Corporation**, Redmond, WA (US)

(72) Inventors: **Paul C. Bornemann**, North Bend, WA (US); **Raj N. Master**, San Jose, CA (US); **Michael Joseph Lane**, Bellevue, WA (US); **Seah Sun Too**, Sammamish, WA (US)

(73) Assignee: **Microsoft Corporation**, Redmond, WA (US)

(\*) Notice: Subject to any disclaimer, the term of this patent is extended or adjusted under 35 U.S.C. 154(b) by 0 days.

(21) Appl. No.: **13/715,133**

(22) Filed: **Dec. 14, 2012**

(30) **Foreign Application Priority Data**

Oct. 17, 2012 (WO) ..... PCT/CN2012/083083

(51) **Int. Cl.**

**B22C 9/06** (2006.01)  
**B22D 17/22** (2006.01)

(52) **U.S. Cl.**

CPC .. **B22C 9/06** (2013.01); **B22D 17/22** (2013.01)  
USPC ..... 164/113; 164/284; 164/303; 164/312;  
164/359

(58) **Field of Classification Search**

USPC ..... 164/359, 113, 133, 284, 303, 312, 337;  
425/555

See application file for complete search history.

(56) **References Cited**

U.S. PATENT DOCUMENTS

4,046,975 A 9/1977 Seeger, Jr.  
4,065,649 A 12/1977 Carter et al.

|             |         |                    |
|-------------|---------|--------------------|
| 4,243,861 A | 1/1981  | Strandwitz         |
| 4,302,648 A | 11/1981 | Sado et al.        |
| 4,317,013 A | 2/1982  | Larson             |
| 4,365,130 A | 12/1982 | Christensen        |
| 4,492,829 A | 1/1985  | Rodrique           |
| 4,527,021 A | 7/1985  | Morikawa et al.    |
| 4,559,426 A | 12/1985 | Van Zeeland et al. |
| 4,588,187 A | 5/1986  | Dell               |
| 4,607,147 A | 8/1986  | Ono et al.         |

(Continued)

FOREIGN PATENT DOCUMENTS

|    |         |         |
|----|---------|---------|
| EP | 2353978 | 8/2011  |
|    | 2378607 | 10/2011 |

(Continued)

OTHER PUBLICATIONS

"Non-Final Office Action", U.S. Appl. No. 13/656,520, (Jun. 5, 2013), 8 pages.

(Continued)

*Primary Examiner* — Kevin P Kerns

*Assistant Examiner* — Kevin E Yoon

(74) *Attorney, Agent, or Firm* — Jeremy Snodgrass; Glen Johnson; Micky Minhas

(57) **ABSTRACT**

Metal alloy injection molding techniques are described. In one or more implementations, these techniques may also include adjustment of injection pressure, configuration of runners, and/or use of vacuum pressure, and so on to encourage flow of the metal alloy through a mold. Techniques are also described that utilize protrusions to counteract thermal expansion and subsequent contraction of the metal alloy upon cooling. Further, techniques are described in which a radius of edges of a feature is configured to encourage flow and reduce voids. A variety of other techniques are also described herein.

**12 Claims, 12 Drawing Sheets**



| (56)                  | References Cited |                     |                   |         |                       |           |
|-----------------------|------------------|---------------------|-------------------|---------|-----------------------|-----------|
| U.S. PATENT DOCUMENTS |                  |                     |                   |         |                       |           |
| 4,651,133 A           | 3/1987           | Ganesan et al.      | 7,639,876 B2      | 12/2009 | Clary et al.          |           |
| 5,220,521 A           | 6/1993           | Kikinis             | 7,656,392 B2      | 2/2010  | Bolender              |           |
| 5,283,559 A           | 2/1994           | Kalendra et al.     | 7,722,792 B2 *    | 5/2010  | Uezaki et al. ....    | 264/328.7 |
| 5,331,443 A           | 7/1994           | Stanisci            | 7,733,326 B1      | 6/2010  | Adiseshan             |           |
| 5,340,528 A *         | 8/1994           | Machida et al. .... | 7,773,076 B2      | 8/2010  | Pittel et al.         |           |
| 5,548,477 A           | 8/1996           | Kumar et al.        | 7,777,972 B1      | 8/2010  | Chen et al.           |           |
| 5,558,577 A           | 9/1996           | Kato                | 7,782,342 B2      | 8/2010  | Koh                   |           |
| 5,618,232 A           | 4/1997           | Martin              | 7,813,715 B2      | 10/2010 | McKillip et al.       |           |
| 5,681,220 A           | 10/1997          | Bertram et al.      | 7,884,807 B2      | 2/2011  | Hovden et al.         |           |
| 5,745,376 A           | 4/1998           | Barker et al.       | D636,397 S        | 4/2011  | Green                 |           |
| 5,748,114 A           | 5/1998           | Koehn               | 7,928,964 B2      | 4/2011  | Kolmykov-Zotov et al. |           |
| 5,781,406 A           | 7/1998           | Hunte               | 7,944,520 B2      | 5/2011  | Ichioka et al.        |           |
| 5,807,175 A           | 9/1998           | Davis et al.        | 7,945,717 B2      | 5/2011  | Rivalsi               |           |
| 5,818,361 A           | 10/1998          | Acevedo             | 7,973,771 B2      | 7/2011  | Geaghan               |           |
| 5,828,770 A           | 10/1998          | Leis et al.         | 7,978,281 B2      | 7/2011  | Vergith et al.        |           |
| 5,874,697 A           | 2/1999           | Selker et al.       | 8,018,386 B2      | 9/2011  | Qi et al.             |           |
| 5,926,170 A           | 7/1999           | Oba                 | 8,026,904 B2      | 9/2011  | Westerman             |           |
| 5,957,191 A *         | 9/1999           | Okada et al. ....   | 8,130,203 B2      | 3/2012  | Westerman             |           |
| 5,971,635 A           | 10/1999          | Wise                | 8,154,524 B2      | 4/2012  | Wilson et al.         |           |
| 6,002,389 A           | 12/1999          | Kasser              | D659,139 S        | 5/2012  | Gengler               |           |
| 6,005,209 A           | 12/1999          | Burleson et al.     | 8,169,421 B2      | 5/2012  | Wright et al.         |           |
| 6,012,714 A           | 1/2000           | Worley et al.       | 8,229,509 B2      | 7/2012  | Paek et al.           |           |
| 6,040,823 A           | 3/2000           | Seffernick et al.   | 8,229,522 B2      | 7/2012  | Kim et al.            |           |
| 6,044,717 A           | 4/2000           | Biegelsen et al.    | 8,654,030 B1      | 2/2014  | Mercer                |           |
| 6,061,644 A           | 5/2000           | Leis                | 2002/0134828 A1   | 9/2002  | Sandbach et al.       |           |
| 6,112,797 A           | 9/2000           | Colson et al.       | 2003/0197687 A1   | 10/2003 | Shetter               |           |
| 6,178,443 B1          | 1/2001           | Lin                 | 2004/0258924 A1   | 12/2004 | Berger et al.         |           |
| 6,254,105 B1          | 7/2001           | Rinde et al.        | 2004/0268000 A1   | 12/2004 | Barker et al.         |           |
| 6,279,060 B1          | 8/2001           | Luke et al.         | 2005/0030728 A1   | 2/2005  | Kawashima et al.      |           |
| 6,329,617 B1          | 12/2001          | Burgess             | 2005/0057515 A1   | 3/2005  | Bathiche              |           |
| 6,344,791 B1          | 2/2002           | Armstrong           | 2005/0059489 A1   | 3/2005  | Kim                   |           |
| 6,380,497 B1          | 4/2002           | Hashimoto et al.    | 2005/0146512 A1   | 7/2005  | Hill et al.           |           |
| 6,437,682 B1          | 8/2002           | Vance               | 2005/0264653 A1   | 12/2005 | Starkweather et al.   |           |
| 6,506,983 B1          | 1/2003           | Babb et al.         | 2005/0264988 A1   | 12/2005 | Nicolosi              |           |
| 6,511,378 B1          | 1/2003           | Bhatt et al.        | 2005/0285703 A1   | 12/2005 | Wheeler et al.        |           |
| 6,532,147 B1          | 3/2003           | Christ, Jr.         | 2006/0049993 A1   | 3/2006  | Lin et al.            |           |
| 6,543,949 B1          | 4/2003           | Ritchey et al.      | 2006/0085658 A1   | 4/2006  | Allen et al.          |           |
| 6,565,439 B2          | 5/2003           | Shinohara et al.    | 2006/0125799 A1   | 6/2006  | Hillis et al.         |           |
| 6,600,121 B1          | 7/2003           | Olodort et al.      | 2006/0154725 A1   | 7/2006  | Glaser et al.         |           |
| 6,603,408 B1          | 8/2003           | Gaba                | 2006/0156415 A1   | 7/2006  | Rubinstein et al.     |           |
| 6,608,664 B1          | 8/2003           | Hasegawa            | 2006/0181514 A1   | 8/2006  | Newman                |           |
| 6,617,536 B2          | 9/2003           | Kawaguchi           | 2006/0195522 A1   | 8/2006  | Miyazaki              |           |
| 6,685,369 B2          | 2/2004           | Lien                | 2006/0254042 A1 * | 11/2006 | Chou et al. ....      | 29/527.1  |
| 6,704,864 B1          | 3/2004           | Philyaw             | 2007/0062089 A1   | 3/2007  | Homer et al.          |           |
| 6,721,019 B2          | 4/2004           | Kono et al.         | 2007/0072474 A1   | 3/2007  | Beasley et al.        |           |
| 6,725,318 B1          | 4/2004           | Sherman et al.      | 2007/0182663 A1   | 8/2007  | Biech                 |           |
| 6,774,888 B1          | 8/2004           | Genduso             | 2007/0200830 A1   | 8/2007  | Yamamoto              |           |
| 6,776,546 B2          | 8/2004           | Kraus et al.        | 2007/0234420 A1   | 10/2007 | Novotney et al.       |           |
| 6,784,869 B1          | 8/2004           | Clark et al.        | 2007/0236408 A1   | 10/2007 | Yamaguchi et al.      |           |
| 6,813,143 B2          | 11/2004          | Makela              | 2007/0247432 A1   | 10/2007 | Oakley                |           |
| 6,819,316 B2          | 11/2004          | Schulz et al.       | 2007/0260892 A1   | 11/2007 | Paul et al.           |           |
| 6,856,506 B2          | 2/2005           | Doherty et al.      | 2007/0283179 A1   | 12/2007 | Burnett et al.        |           |
| 6,861,961 B2          | 3/2005           | Sandbach et al.     | 2008/005423 A1    | 1/2008  | Jacobs et al.         |           |
| 6,898,315 B2          | 5/2005           | Guha                | 2008/0104437 A1   | 5/2008  | Lee                   |           |
| 6,914,197 B2          | 7/2005           | Doherty et al.      | 2008/0151478 A1   | 6/2008  | Chern                 |           |
| 6,950,950 B2          | 9/2005           | Sawyers et al.      | 2008/0158185 A1   | 7/2008  | Westerman             |           |
| 6,970,957 B1          | 11/2005          | Oshins et al.       | 2008/0167832 A1   | 7/2008  | Soss                  |           |
| 6,976,799 B2          | 12/2005          | Kim et al.          | 2008/0238884 A1   | 10/2008 | Harish                |           |
| 7,051,149 B2          | 5/2006           | Wang et al.         | 2008/0253822 A1   | 10/2008 | Matias                |           |
| 7,083,295 B1          | 8/2006           | Hanna               | 2008/0309636 A1   | 12/2008 | Feng et al.           |           |
| 7,091,436 B2          | 8/2006           | Serban              | 2008/0316002 A1   | 12/2008 | Brunet et al.         |           |
| 7,106,222 B2          | 9/2006           | Ward et al.         | 2008/0320190 A1   | 12/2008 | Lydon et al.          |           |
| 7,123,292 B1          | 10/2006          | Seeger et al.       | 2009/009476 A1    | 1/2009  | Daley, III            |           |
| 7,194,662 B2          | 3/2007           | Do et al.           | 2009/0073060 A1   | 3/2009  | Shimasaki et al.      |           |
| 7,213,991 B2          | 5/2007           | Chapman et al.      | 2009/0073957 A1   | 3/2009  | Newland et al.        |           |
| 7,277,087 B2          | 10/2007          | Hill et al.         | 2009/0079639 A1   | 3/2009  | Hotta et al.          |           |
| 7,447,934 B2          | 11/2008          | Dasari et al.       | 2009/0127005 A1   | 5/2009  | Zachut et al.         |           |
| 7,469,386 B2          | 12/2008          | Bear et al.         | 2009/0140985 A1   | 6/2009  | Liu                   |           |
| 7,499,037 B2          | 3/2009           | Lube                | 2009/0163147 A1   | 6/2009  | Steigerwald et al.    |           |
| 7,502,803 B2          | 3/2009           | Culter et al.       | 2009/0251008 A1   | 10/2009 | Sugaya                |           |
| 7,542,052 B2          | 6/2009           | Solomon et al.      | 2009/0262492 A1   | 10/2009 | Whitchurch et al.     |           |
| 7,558,594 B2          | 7/2009           | Wilson              | 2009/0303137 A1   | 12/2009 | Kusaka et al.         |           |
| 7,559,834 B1          | 7/2009           | York                | 2009/0303204 A1   | 12/2009 | Nasiri et al.         |           |
| 7,620,244 B1          | 11/2009          | Collier             | 2009/0320244 A1   | 12/2009 | Lin                   |           |
| 7,636,921 B2          | 12/2009          | Louie               | 2009/0321490 A1   | 12/2009 | Groene et al.         |           |

(56)

## References Cited

## U.S. PATENT DOCUMENTS

|                 |         |                   |                 |         |                   |
|-----------------|---------|-------------------|-----------------|---------|-------------------|
| 2010/0001963 A1 | 1/2010  | Doray et al.      | 2012/0024682 A1 | 2/2012  | Huang et al.      |
| 2010/0026656 A1 | 2/2010  | Hotelling et al.  | 2012/0026048 A1 | 2/2012  | Vazquez et al.    |
| 2010/0038821 A1 | 2/2010  | Jenkins et al.    | 2012/0044179 A1 | 2/2012  | Hudson            |
| 2010/0045540 A1 | 2/2010  | Lai et al.        | 2012/0047368 A1 | 2/2012  | Chinn et al.      |
| 2010/0045609 A1 | 2/2010  | Do et al.         | 2012/0050975 A1 | 3/2012  | Garelli et al.    |
| 2010/0045633 A1 | 2/2010  | Gettemy           | 2012/0075249 A1 | 3/2012  | Hoch              |
| 2010/0051356 A1 | 3/2010  | Stern et al.      | 2012/0081316 A1 | 4/2012  | Sirpal et al.     |
| 2010/0051432 A1 | 3/2010  | Lin et al.        | 2012/0092279 A1 | 4/2012  | Martin            |
| 2010/0053534 A1 | 3/2010  | Hsieh et al.      | 2012/0094257 A1 | 4/2012  | Pillischer et al. |
| 2010/0077237 A1 | 3/2010  | Sawyers           | 2012/0099749 A1 | 4/2012  | Rubin et al.      |
| 2010/0081377 A1 | 4/2010  | Chatterjee et al. | 2012/0115553 A1 | 5/2012  | Mahe et al.       |
| 2010/0085321 A1 | 4/2010  | Pundsack          | 2012/0117409 A1 | 5/2012  | Lee et al.        |
| 2010/0103112 A1 | 4/2010  | Yoo et al.        | 2012/0127118 A1 | 5/2012  | Nolting et al.    |
| 2010/0149111 A1 | 6/2010  | Olien             | 2012/0133561 A1 | 5/2012  | Konanur et al.    |
| 2010/0149134 A1 | 6/2010  | Westerman et al.  | 2012/0140396 A1 | 6/2012  | Zeliff et al.     |
| 2010/0156798 A1 | 6/2010  | Archer            | 2012/0145525 A1 | 6/2012  | Ishikawa          |
| 2010/0161522 A1 | 6/2010  | Tirpak et al.     | 2012/0162693 A1 | 6/2012  | Ito               |
| 2010/0164857 A1 | 7/2010  | Liu et al.        | 2012/0182242 A1 | 7/2012  | Lindahl et al.    |
| 2010/0171891 A1 | 7/2010  | Kaji et al.       | 2012/0194393 A1 | 8/2012  | Uttermann et al.  |
| 2010/0174421 A1 | 7/2010  | Tsai et al.       | 2012/0194448 A1 | 8/2012  | Rothkopf          |
| 2010/0180063 A1 | 7/2010  | Ananny et al.     | 2012/0223866 A1 | 9/2012  | Ayala et al.      |
| 2010/0188299 A1 | 7/2010  | Rinehart et al.   | 2012/0224073 A1 | 9/2012  | Miyahara          |
| 2010/0206614 A1 | 8/2010  | Park et al.       | 2012/0235635 A1 | 9/2012  | Sato              |
| 2010/0206644 A1 | 8/2010  | Yeh               | 2012/0246377 A1 | 9/2012  | Bhesania          |
| 2010/0214257 A1 | 8/2010  | Wussler et al.    | 2012/0256959 A1 | 10/2012 | Ye et al.         |
| 2010/0222110 A1 | 9/2010  | Kim et al.        | 2012/0274811 A1 | 11/2012 | Bakin             |
| 2010/0231556 A1 | 9/2010  | Mines et al.      | 2012/0300275 A1 | 11/2012 | Vilardell et al.  |
| 2010/0238075 A1 | 9/2010  | Pourseyed         | 2013/0063873 A1 | 3/2013  | Wodrich et al.    |
| 2010/0250988 A1 | 9/2010  | Okuda et al.      | 2013/0227836 A1 | 9/2013  | Whitt, III        |
| 2010/0274932 A1 | 10/2010 | Kose              | 2013/0228435 A1 | 9/2013  | Whitt, III        |
| 2010/0279768 A1 | 11/2010 | Huang et al.      | 2013/0229356 A1 | 9/2013  | Marwah            |
| 2010/0289457 A1 | 11/2010 | Onnerud et al.    | 2013/0229366 A1 | 9/2013  | Dighde            |
| 2010/0295812 A1 | 11/2010 | Burns et al.      | 2013/0229759 A1 | 9/2013  | Whitt, III        |
| 2010/0302378 A1 | 12/2010 | Marks et al.      | 2013/0335902 A1 | 12/2013 | Campbell          |
| 2010/0304793 A1 | 12/2010 | Kim               |                 |         |                   |
| 2010/0306538 A1 | 12/2010 | Thomas et al.     |                 |         |                   |
| 2010/0308778 A1 | 12/2010 | Yamazaki et al.   |                 |         |                   |
| 2010/0308844 A1 | 12/2010 | Day et al.        |                 |         |                   |
| 2010/0315348 A1 | 12/2010 | Jellicoe et al.   |                 |         |                   |
| 2010/0325155 A1 | 12/2010 | Skinner et al.    |                 |         |                   |
| 2010/0331059 A1 | 12/2010 | Apgar et al.      |                 |         |                   |
| 2011/0012873 A1 | 1/2011  | Prest et al.      |                 |         |                   |
| 2011/0019123 A1 | 1/2011  | Prest et al.      |                 |         |                   |
| 2011/0031287 A1 | 2/2011  | Le Gette et al.   |                 |         |                   |
| 2011/0037721 A1 | 2/2011  | Cranfill et al.   |                 |         |                   |
| 2011/0043990 A1 | 2/2011  | Mickey et al.     |                 |         |                   |
| 2011/0060926 A1 | 3/2011  | Brooks et al.     |                 |         |                   |
| 2011/0069148 A1 | 3/2011  | Jones et al.      |                 |         |                   |
| 2011/0074688 A1 | 3/2011  | Hull et al.       |                 |         |                   |
| 2011/0102326 A1 | 5/2011  | Casparian et al.  |                 |         |                   |
| 2011/0102356 A1 | 5/2011  | Kempainen et al.  |                 |         |                   |
| 2011/0134032 A1 | 6/2011  | Chiu et al.       |                 |         |                   |
| 2011/0157087 A1 | 6/2011  | Kanehira et al.   |                 |         |                   |
| 2011/0163955 A1 | 7/2011  | Nasiri et al.     |                 |         |                   |
| 2011/0164370 A1 | 7/2011  | McClure et al.    |                 |         |                   |
| 2011/0167181 A1 | 7/2011  | Minoo et al.      |                 |         |                   |
| 2011/0167287 A1 | 7/2011  | Walsh et al.      |                 |         |                   |
| 2011/0167391 A1 | 7/2011  | Momeyer et al.    |                 |         |                   |
| 2011/0167992 A1 | 7/2011  | Eventoff et al.   |                 |         |                   |
| 2011/0179864 A1 | 7/2011  | Raasch et al.     |                 |         |                   |
| 2011/0184646 A1 | 7/2011  | Wong et al.       |                 |         |                   |
| 2011/0193787 A1 | 8/2011  | Morishige et al.  |                 |         |                   |
| 2011/0205372 A1 | 8/2011  | Miramontes        |                 |         |                   |
| 2011/0227913 A1 | 9/2011  | Hyndman           |                 |         |                   |
| 2011/0242138 A1 | 10/2011 | Tribble           |                 |         |                   |
| 2011/0248920 A1 | 10/2011 | Larsen            |                 |         |                   |
| 2011/0261001 A1 | 10/2011 | Liu               |                 |         |                   |
| 2011/0290686 A1 | 12/2011 | Huang             |                 |         |                   |
| 2011/0297566 A1 | 12/2011 | Gallagher et al.  |                 |         |                   |
| 2011/0304577 A1 | 12/2011 | Brown             |                 |         |                   |
| 2011/0316807 A1 | 12/2011 | Corrion           |                 |         |                   |
| 2012/0007821 A1 | 1/2012  | Zaliva            |                 |         |                   |
| 2012/0011462 A1 | 1/2012  | Westerman et al.  |                 |         |                   |
| 2012/0013519 A1 | 1/2012  | Hakansson et al.  |                 |         |                   |
| 2012/0023459 A1 | 1/2012  | Westerman         |                 |         |                   |

## FOREIGN PATENT DOCUMENTS

|    |               |         |
|----|---------------|---------|
| JP | 10326124      | 12/1998 |
| WO | WO-2008055039 | 5/2008  |
| WO | WO-2010105272 | 9/2010  |

## OTHER PUBLICATIONS

“PCT Search Report and Written Opinion”, Application No. PCT/US2013/028948, (Jun. 21, 2013), 11 pages.

“Restriction Requirement”, U.S. Appl. No. 13/715,229, (Aug. 13, 2013), 7 pages.

“Notice of Allowance”, U.S. Appl. No. 13/656,520, (Oct. 2, 2013), 5 pages.

“Accessing Device Sensors”, retrieved from <<https://developer.palm.com/content/api/dev-guide/pdk/accessing-device-sensors.html>> on May 25, 2012, 4 pages.

“ACPI Docking for Windows Operating Systems”, Retrieved from: <<http://www.scritube.com/limba/ngleza/software/ACPI-Docking-for-Windows-Opera331824193.php>> on Jul. 6, 2012, 10 pages.

“Cholesteric Liquid Crystal”, Retrieved from: <[http://en.wikipedia.org/wiki/Cholesteric\\_liquid\\_crystal](http://en.wikipedia.org/wiki/Cholesteric_liquid_crystal)> on Aug. 6, 2012, (Jun. 10, 2012), 2 pages.

“Cirago Slim Case®—Protective case with built-in kickstand for your iPhone 5®”, Retrieved from <<http://cirago.com/wordpress/wp-content/uploads/2012/10/1pc1500brochure1.pdf>> on Jan. 29, 2013, 1 page.

“DR2PA”, retrieved from <[http://www.architainment.co.uk/wp-content/uploads/2012/08/DR2PA-AU-US-size-Data-Sheet-Rev-H\\_LOGO.pdf](http://www.architainment.co.uk/wp-content/uploads/2012/08/DR2PA-AU-US-size-Data-Sheet-Rev-H_LOGO.pdf)> on Sep. 17, 2012, 4 pages.

“First One Handed Fabric Keyboard with Bluetooth Wireless Technology”, Retrieved from: <<http://press.xtvworld.com/article3817.html>> on May 8, 2012, (Jan. 6, 2005), 2 pages.

“Force and Position Sensing Resistors: An Emerging Technology”, *Interlink Electronics*, Available at <[http://staff.science.uva.nl/~vlaander/docu/FSR/An\\_Exploring\\_Technology.pdf](http://staff.science.uva.nl/~vlaander/docu/FSR/An_Exploring_Technology.pdf)>, (Feb. 1990), pp. 1-6 .

“Frogpad Introduces Wearable Fabric Keyboard with Bluetooth Technology”, Retrieved from: <<http://www.geekzone.co.nz/content.asp?contentid=3898>> on May 7, 2012, (Jan. 7, 2005), 3 pages.

(56)

**References Cited**

## OTHER PUBLICATIONS

- “How to Use the iPad’s Onscreen Keyboard”, Retrieved from <<http://www.dummies.com/how-to/content/how-to-use-the-ipads-onscreen-keyboard.html>> on Aug. 28, 2012, 3 pages.
- “i-Interactor electronic pen”, Retrieved from: <[http://www.alibaba.com/product-gs/331004878/i\\_Interactor\\_electronic\\_pen.html](http://www.alibaba.com/product-gs/331004878/i_Interactor_electronic_pen.html)> on Jun. 19, 2012, 5 pages.
- “Incipio LG G-Slate Premium Kickstand Case—Black Nylon”, Retrieved from: <<http://www.amazon.com/Incipio-G-Slate-Premium-Kickstand-Case/dp/B004ZKP916>> on May 8, 2012, 4 pages.
- “Membrane Keyboards & Membrane Keypads”, Retrieved from: <<http://www.pannam.com/>> on May 9, 2012,(Mar. 4, 2009), 2 pages.
- “Motion Sensors”, *Android Developers*, retrieved from <[http://developer.android.com/guide/topics/sensors/sensors\\_motion.html](http://developer.android.com/guide/topics/sensors/sensors_motion.html)> on May 25, 2012, 7 pages.
- “MPC Fly Music Production Controller”, *AKAI Professional*, Retrieved from: <<http://www.akaiprompc.com/mpc-fly>> on Jul. 9, 2012, 4 pages.
- “Ni Releases New Maschine & Maschine Mikro”, Retrieved from <<http://www.djbooth.net/index/dj-equipment/entry/ni-releases-new-maschine-mikro/>> on Sep. 17, 2012, 19 pages.
- “Non-Final Office Action”, U.S. Appl. No. 13/471,001, (Feb. 19, 2013),15 pages.
- “Non-Final Office Action”, U.S. Appl. No. 13/471,139, (Mar. 21, 2013),12 pages.
- “Non-Final Office Action”, U.S. Appl. No. 13/471,202, (Feb. 11, 2013),10 pages.
- “Non-Final Office Action”, U.S. Appl. No. 13/471,336, (Jan. 18, 2013),14 pages.
- “Non-Final Office Action”, U.S. Appl. No. 13/651,195, (Jan. 2, 2013),14 pages.
- “Non-Final Office Action”, U.S. Appl. No. 13/651,232, (Jan. 17, 2013),15 pages.
- “Non-Final Office Action”, U.S. Appl. No. 13/651,272, (Feb. 12, 2013),10 pages.
- “Non-Final Office Action”, U.S. Appl. No. 13/651,287, (Jan. 29, 2013),13 pages.
- “Non-Final Office Action”, U.S. Appl. No. 13/651,304, (Mar. 22, 2013), 9 pages.
- “Non-Final Office Action”, U.S. Appl. No. 13/651,327, (Mar. 22, 2013), 6 pages.
- “Non-Final Office Action”, U.S. Appl. No. 13/651,871, (Mar. 18, 2013),14 pages.
- “Non-Final Office Action”, U.S. Appl. No. 13/651,976, (Feb. 22, 2013),16 pages.
- “Non-Final Office Action”, U.S. Appl. No. 13/653,321, (Feb. 1, 2013),13 pages.
- “Non-Final Office Action”, U.S. Appl. No. 13/653,682, (Feb. 7, 2013),11 pages.
- “Non-Final Office Action”, U.S. Appl. No. 13/656,520, (Feb. 1, 2013),15 pages.
- “Notice of Allowance”, U.S. Appl. No. 13/470,633, (Mar. 22, 2013), 7 pages.
- “On-Screen Keyboard for Windows 7, Vista, XP with Touchscreen”, Retrieved from <<http://www.comfort-software.com/on-screen-keyboard.html>> on Aug. 28, 2012, (Feb. 2, 2011), 3 pages.
- “Position Sensors”, *Android Developers*, retrieved from <[http://developer.android.com/guide/topics/sensors/sensors\\_position.html](http://developer.android.com/guide/topics/sensors/sensors_position.html)> on May 25, 2012, 5 pages.
- “Reflex LCD Writing Tablets”, retrieved from <<http://www.kentdisplays.com/products/lcdwritingtablets.html>> on Jun. 27, 2012, 3 pages.
- “Restriction Requirement”, U.S. Appl. No. 13/471,139, (Jan. 17, 2013), 7 pages.
- “Restriction Requirement”, U.S. Appl. No. 13/651,304, (Jan. 18, 2013), 7 pages.
- “Restriction Requirement”, U.S. Appl. No. 13/651,726, (Feb. 22, 2013), 6 pages.
- “Restriction Requirement”, U.S. Appl. No. 13/651,871, (Feb. 7, 2013), 6 pages.
- “SMART Board™ Interactive Display Frame Pencil Pack”, Available at <[http://downloads01.smarttech.com/media/sitecore/en/support/product/sbfpd/400series\(interactivedisplayframes\)/guides/smartboardinteractivedisplayframepencilpackv12mar09.pdf](http://downloads01.smarttech.com/media/sitecore/en/support/product/sbfpd/400series(interactivedisplayframes)/guides/smartboardinteractivedisplayframepencilpackv12mar09.pdf)>,(2009), 2 pages.
- “SoIRxTM E-Series Multidirectional Phototherapy ExpandableTM 2-Bulb Full Body Panel System”, Retrieved from: <[http://www.solarcsystems.com/us\\_multidirectional\\_uv\\_light\\_therapy\\_1\\_intro.html](http://www.solarcsystems.com/us_multidirectional_uv_light_therapy_1_intro.html)> on Jul. 25, 2012,(2011), 4 pages.
- “The Microsoft Surface Tablets Comes With Impressive Design and Specs”, Retrieved from <<http://microsofttabletreview.com/the-microsoft-surface-tablets-comes-with-impressive-design-and-specs>> on Jan. 30, 2013, (Jun. 2012), 2 pages.
- “Tilt Shift Lenses: Perspective Control”, retrieved from <http://www.cambridgeincolour.com/tutorials/tilt-shift-lenses1.htm>, (Mar. 28, 2008),11 Pages.
- “Virtualization Getting Started Guide”, *Red Hat Enterprise Linux 6, Edition 0.2*, retrieved from <[http://docs.redhat.com/docs/en-US/Red\\_Hat\\_Enterprise\\_Linux/6/html-single/Virtualization\\_Getting\\_Started\\_Guide/index.html](http://docs.redhat.com/docs/en-US/Red_Hat_Enterprise_Linux/6/html-single/Virtualization_Getting_Started_Guide/index.html)> on Jun. 13, 2012, 24 pages.
- “What is Active Alignment?”, [http://www.kasalis.com/active\\_alignment.html](http://www.kasalis.com/active_alignment.html), retrieved on Nov. 22, 2012, 2 Pages.
- Block, Steve et al., “DeviceOrientation Event Specification”, *W3C, Editor’s Draft*, retrieved from <<https://developer.palm.com/content/api/dev-guide/pdk/accessing-device-sensors.html>> on May 25, 2012,(Jul. 12, 2011), 14 pages.
- Brown, Rich “Microsoft Shows Off Pressure-Sensitive Keyboard”, retrieved from <[http://news.cnet.com/8301-17938\\_105-10304792-1.html](http://news.cnet.com/8301-17938_105-10304792-1.html)> on May 7, 2012, (Aug. 6, 2009), 2 pages.
- Butler, Alex et al., “SideSight: Multi-“touch” Interaction around Small Devices”, *In the proceedings of the 21st annual ACM symposium on User interface software and technology.*, retrieved from <[http://research.microsoft.com/pubs/132534/sidesight\\_crv3.pdf](http://research.microsoft.com/pubs/132534/sidesight_crv3.pdf)> on May 29, 2012,(Oct. 19, 2008), 4 pages.
- Crider, Michael “Sony Slate Concept Tablet “Grows” a Kickstand”, Retrieved from: <<http://androidcommunity.com/sony-slate-concept-tablet-grows-a-kickstand-20120116/>> on May 4, 2012,(Jan. 16, 2012), 9 pages.
- Das, Apurba et al., “Study of Heat Transfer through Multilayer Clothing Assemblies: A Theoretical Prediction”, Retrieved from <[http://www.autexrj.com/cms/zalaczone\\_pliki/5\\_11.pdf](http://www.autexrj.com/cms/zalaczone_pliki/5_11.pdf)>, (Jun. 2011), 7 pages.
- Dietz, Paul H., et al., “A Practical Pressure Sensitive Computer Keyboard”, In Proceedings of UIST 2009,(Oct. 2009), 4 pages.
- Glatt, Jeff “Channel and Key Pressure (Aftertouch)”, Retrieved from: <<http://home.roadrunner.com/~jgglatt/tutr/touch.htm>> on Jun. 11, 2012, 2 pages.
- Hanlon, Mike “ElekTex Smart Fabric Keyboard Goes Wireless”, Retrieved from: <<http://www.gizmag.com/go/5048/>> on May 7, 2012,(Jan. 15, 2006), 5 pages.
- Iwase, Eiji “Multistep Sequential Batch Assembly of Three-Dimensional Ferromagnetic Microstructures with Elastic Hinges”, Retrieved at <<http://ieeexplore.ieee.org/stamp/stamp.jsp?tp=&arnumber=15498611>> *Proceedings: Journal of Microelectromechanical Systems*, (Dec. 2005), 7 pages.
- Kaur, Sukhmani “Vincent Liew’s redesigned laptop satisfies ergonomic needs”, Retrieved from: <<http://www.designbuzz.com/entry/vincent-liew-s-redesigned-laptop-satisfies-ergonomic-needs/>> on Jul. 27, 2012,(Jun. 21, 2010), 4 pages.
- Khunontong, Puttachat et al., “Fabrication of Molded Interconnection Devices by Ultrasonic Hot Embossing on Thin Polymer Films”, *IEEE Transactions on Electronics Packaging Manufacturing*, vol. 32, No. 3,(Jul. 2009), pp. 152-156.
- Li, et al., “Characteristic Mode Based Tradeoff Analysis of Antenna-Chassis Interactions for Multiple Antenna Terminals”, *In IEEE Transactions on Antennas and Propagation*, Retrieved from <<http://ieeexplore.ieee.org/stamp/stamp.jsp?tp=&arnumber=6060882>>,(Feb. 2012),13 pages.
- Linderholm, Owen “Logitech Shows Cloth Keyboard for PDAs”, Retrieved from: <[http://www.pcworld.com/article/89084/logitech\\_shows\\_cloth\\_keyboard\\_for\\_pdas.html](http://www.pcworld.com/article/89084/logitech_shows_cloth_keyboard_for_pdas.html)> on May 7, 2012,(Mar. 15, 2002), 5 pages.

(56)

**References Cited**

## OTHER PUBLICATIONS

- McLellan, Charles "Eleksen Wireless Fabric Keyboard: a first look", Retrieved from: <<http://www.zdnetasia.com/eleksen-wireless-fabric-keyboard-a-first-look-40278954.htm>> on May 7, 2012,(Jul. 17, 2006), 9 pages.
- Piltch, Avram "ASUS Eee Pad Slider SL101 Review ", Retrieved from <<http://www.laptopmag.com/review/tablets/asus-eee-pad-slider-sl101.aspx>>, (Sep. 22, 2011), 5 pages.
- Post, E.R. et al., "E-Broidery: Design and Fabrication of Textile-Based Computing", IBM Systems Journal, vol. 39, Issue 3 & 4,(Jul. 2000), pp. 840-860.
- Purcher, Jack "Apple is Paving the Way for a New 3D GUI for IOS Devices", Retrieved from: <<http://www.patentlyapple.com/patently-apple/2012/01/apple-is-paving-the-way-for-a-new-3d-gui-for-ios-devices.html>> on Jun. 4, 2012,(Jan. 12, 2012),15 pages.
- Qin, Yongqiang et al., "pPen: Enabling Authenticated Pen and Touch Interaction on Tabletop Surfaces", *In Proceedings of ITS 2010*, Available at <<http://www.dfk1.de/its2010/papers/pdf/po172.pdf>>,(Nov. 2010), pp. 283-284.
- Sumimoto, Mark "Touch & Write: Surface Computing With Touch and Pen Input", Retrieved from: <<http://www.gottabemobile.com/2009/08/07/touch-write-surface-computing-with-touch-and-pen-input/>> on Jun. 19, 2012,(Aug. 7, 2009), 4 pages.
- Takamatsu, Seiichi et al., "Flexible Fabric Keyboard with Conductive Polymer-Coated Fibers", In Proceedings of Sensors 2011,(Oct. 28, 2011), 4 pages.
- Vallith, G T., "Design of Hologram for Brightness Enhancement in Color LCDs", Retrieved from <[http://www.loreti.it/Download/PDF/LCD/44\\_05.pdf](http://www.loreti.it/Download/PDF/LCD/44_05.pdf)> on Sep. 17, 2012, 5 pages.
- Williams, Jim "A Fourth Generation of LCD Backlight Technology", Retrieved from <<http://cds.linear.com/docs/Application%20Note/an65f.pdf>>, (Nov. 1995),124 pages.
- Zhang, et al., "Model-Based Development of Dynamically Adaptive Software", *In Proceedings of ICSE 2006*, Available at <<http://www.irisa.fr/lande/lande/icse-proceedings/icse/p371.pdf>>,(May 20, 2006), pp. 371-380.
- "Corrected Notice of Allowance", U.S. Appl. No. 13/656,520, Jan. 16, 2014, 3 pages.
- "International Search Report and Written Opinion", Application No. PCT/US2013/065154, Feb. 5, 2014, 10 pages.
- "Non-Final Office Action", U.S. Appl. No. 13/599,635, Feb. 25, 2014, 13 pages.

\* cited by examiner



Fig. 1



*Fig. 2*



*Fig. 3*



Fig. 4



Fig. 5



*Fig. 6*



Fig. 7



*Fig. 8*

*Fig. 9*

1000



Fig. 10

1100 →



Fig. 11

1200



1202

Inject a metal alloy into a mold having a plurality of molding portions that define a cavity that corresponds to an article to be molded, the mold defining a portion of the cavity that defines a feature for the article having a thickness that is greater than a thickness of an area of the article defined by the cavity that is proximal to the feature; and a protrusion for the article aligned as substantially opposing the feature, the protrusion being sized such that upon solidifying of the metal alloy that forms the article, the protrusion reduces an effect of thermal expansion on a portion of the article that is aligned as substantially opposing the feature

1204

Remove the metal alloy from the cavity of the mold after solidifying of the metal alloy within the mold

Fig. 12

1300

1302

Form a mold comprising a plurality of molding portions to form an article using a metal alloy that is defined in the mold using a cavity

1304

Form a portion of the cavity that defines a feature for the article having a thickness that is greater than a thickness of an area of the article defined by the cavity that is proximal to the feature

1306

Form a protrusion for the article aligned on a side of the cavity that is opposite to a side including the feature, the protrusion being sized as being proportional to the thickness of the feature such that upon solidifying of the metal alloy that forms the article, the protrusion reduces an effect of thermal expansion on the side of the article that is opposite to the feature

*Fig. 13*

1400

1402

Inject a metal alloy into a mold having a plurality of molding portions that define a cavity that corresponds to an article to be molded including walls with a thickness of less than one millimeter with one or more features disposed thereon having edges with a radius of at least 0.6 millimeter

1404

Machine at least a portion of the radius of the edge to define the feature of the article after removal of the metal alloy from the cavity

*Fig. 14*

## METAL ALLOY INJECTION MOLDING PROTRUSIONS

### RELATED MATTERS

This application claims priority under 35 USC 119(b) to International Application No. PCT/CN2012/083083 filed Oct. 17, 2012, the disclosure of which is incorporated in its entirety.

### BACKGROUND

Injection molding is a manufacturing process that is conventionally utilized to form articles from plastic. This may include use of thermoplastic and thermosetting plastic materials to form an article, such as a toy, car parts, and so on.

Techniques were subsequently developed to use injection molding for materials other than plastic, such as metal alloys. However, characteristics of the metal alloys could limit use of conventional injection molding techniques to small articles such as watch parts due to complications caused by these characteristics, such as to flow, thermal expansion, and so on.

### SUMMARY

Metal alloy injection molding techniques are described. In one or more implementations, these techniques may include adjustment of injection pressure, configuration of runners, and/or use of vacuum pressure, and so on to encourage flow of the metal alloy through a mold. Techniques are also described that utilize protrusions to counteract thermal expansion and subsequent contraction of the metal alloy upon cooling. Further, techniques are described in which a radius of edges of a feature is configured to encourage flow and reduce voids. A variety of other techniques are also described herein.

This Summary is provided to introduce a selection of concepts in a simplified form that are further described below in the Detailed Description. This Summary is not intended to identify key features or essential features of the claimed subject matter, nor is it intended to be used as an aid in determining the scope of the claimed subject matter.

### BRIEF DESCRIPTION OF THE DRAWINGS

The detailed description is described with reference to the accompanying figures. In the figures, the left-most digit(s) of a reference number identifies the figure in which the reference number first appears. The use of the same reference numbers in different instances in the description and the figures may indicate similar or identical items. Entities represented in the figures may be indicative of one or more entities and thus reference may be made interchangeably to single or plural forms of the entities in the discussion.

FIG. 1 is an illustration of an environment in an example implementation that is operable to employ injection molding techniques described herein.

FIG. 2 depicts an example implementation in which features of an article molded using a system of FIG. 1 is shown.

FIG. 3 depicts an example implementation in which a cavity defined by mold portions may be shaped to form a wall and features of FIG. 2.

FIG. 4 depicts a system in an example implementation in which an injection distribution device is used to physically couple an outflow of injected metal alloy from an injection device to a mold of a molding device.

FIG. 5 depicts an example implementation showing comparison of respective cross sections of the runner and the plurality of sub-runners of FIG. 4.

FIG. 6 depicts a system in an example implementation in which a vacuum device is employed to create negative pressure inside a cavity of the mold to promote flow of the metal alloy.

FIG. 7 depicts a system in an example implementation in which a mold includes one or more overflows to bias a flow of metal alloy through a mold.

FIG. 8 depicts an example implementation in which a protrusion is utilized to reduce an effect of thermal expansion caused by varying degrees of thickness of an article to be molded.

FIG. 9 depicts an example implementation in which a mold is employed that includes edges configured to reduce voids.

FIG. 10 is a flow diagram depicting a procedure in an example implementation in which an article is injected molded using a mold that employs overflows.

FIG. 11 is a flow diagram depicting a procedure in an example implementation in which a mold is formed that employs overflows.

FIG. 12 is a flow diagram depicting a procedure in an example implementation in which a protrusion is formed to at least partially counteract thermal expansion of the metal alloy and subsequent contraction caused by cooling of the metal alloy.

FIG. 13 is a flow diagram depicting a procedure in an example implementation in which a mold is formed that is configured to form a protrusion on an article to counteract an effect of thermal expansion.

FIG. 14 is a flow diagram depicting a procedure in an example implementation in which a radius is employed to limit formation of voids of the article.

### DETAILED DESCRIPTION

#### Overview

Conventional injection molding techniques could encounter complications when utilized for a metal alloy. For example, characteristics of the metal alloy may make these conventional techniques unsuitable to make articles over a relatively short length (e.g., larger than a watch part), that are relatively thin (e.g., less than one millimeter), and so on due to such characteristics of thermal expansion, cooling in a mold, and so forth.

Metal alloy injection molding techniques are described. In one or more implementations, techniques are described that may be utilized to support injection molding of a metal alloy, such as a metal alloy that is comprised primarily of magnesium. These techniques include configuration of runners used to fill a cavity of a mold such that a rate of flow is not slowed by the runners, such as to match an overall size of branches of a runner to a runner from which they branch.

In another example, injection pressure and vacuum pressure may be arranged to encourage flow through an entirety of a cavity that is used to form an article. The vacuum pressure, for instance, may be used to bias flow toward portions of the cavity that otherwise may be difficult to fill. This biasing may also be performed using overflows to encourage flow toward these areas, such as areas of the cavity that are feature rich and thus may be difficult to fill using conventional techniques.

In a further example, protrusions may be formed to counteract effects of thermal expansion on an article to be molded.

The protrusions, for instance, may be sized to counteract shrinkage caused by a thickness of a feature after the metal alloy cools in the mold. In this way, the protrusions may be

used to form a substantially flat surface even though features may be disposed on an opposing side of the surface.

In yet another example, a radius may be employed by features to encourage fill and reduce voids in an article. In a relatively thin article (e.g., less than one millimeter), for instance, sharp corners may cause voids at the corners due to turbulence and other factors encountered in the injection of the metal alloy into a mold. Accordingly, a radius may be utilized that is based at least in part on a thickness of the article to encourage flow and reduce voids. A variety of other examples are also contemplated, further discussion of which may be found in relation to the following sections.

In the following discussion, an example environment is first described that may employ the techniques described herein. Example procedures are then described which may be performed in the example environment as well as other environments. Consequently, performance of the example procedures is not limited to the example environment and the example environment is not limited to performance of the example procedures. It should be readily apparent that these technique may be combined, separated, and so on.

#### Example Environment

FIG. 1 is an illustration of an environment in an example implementation showing a system 100 that is operable to employ injection mold techniques described herein. The illustrated environment includes a computing device 102 that is communicatively coupled to an injection device 104 and a molding device 106. Although illustrated separately, the functionality represented by these apparatus may be combined, further divided, and so on.

The computing device 102 is illustrated as including an injection molding control module 108, which is representative of functionality to control operation of the injection device 104 and molding device 106. The injection molding control module 108, for instance, may utilize one or more instructions 110 stored on a computer-readable storage media 112. The one or more instructions 110 may then be used to control operation of the injection device 104 and molding device 106 to form an article using injection molding.

The injection device 104, for instance, may include an injection control module 116 to control heating and injection of a metal alloy 118 that is to be injected into a mold 120 of the molding device 106. Injection device 104, for instance, may include a heating element to heat and liquefy the metal alloy 118, such as to melt a metal alloy comprised primarily of magnesium to approximately six hundred and fifty degrees Celsius. The injection device 104 may then employ an injector (e.g., a plunger or screw type injector) to inject the metal alloy 118 in liquid form under pressure into the mold 120 of the molding device, such as at approximately forty mPa although other pressures are also contemplated.

The molding device 106 is illustrated as including a mold control module 122, which is representative of functionality to control operation of the mold 120. The mold 120, for instance, may a plurality of mold portions 124, 126. The mold portions 124, 126 when disposed proximal to each other form a cavity 128 that defines the article 114 to be molded. The mold portions 124, 126 may then be moved apart to remove the article 114 from the mold 120.

As previously described, conventional techniques may encounter complications when used to mold an article 114 using a metal alloy 118. For example, an article 114 having walls with a thickness of less than one millimeter may make it difficult to fill an entirety of the cavity 128 to form the article 114 as the metal alloy 118 may not readily flow through the cavity 128 before cooling. This may be further complicated when the article 114 includes a variety of different features

that are to be formed on part of the wall, as further described as follows and shown in a corresponding figure.

FIG. 2 depicts an example implementation 200 in which features of an article molded using the system 100 of FIG. 1 is shown. In this example, the article 114 is configured to form part of a housing for a computing device in a hand held form factor, e.g., tablet, mobile phone, game device, music device, and so on.

The article 114 in this instance includes portions that define a wall 202 of the article 114. Features 204, 206 are also included that extend away from the wall 202 and thus have a thickness that is greater than the wall. Additionally, the features 204, 206 may have a width that is considered relatively thin in comparison with this thickness. Accordingly, in form factors in which the wall is also considered thin (e.g., less than one millimeter) it may be difficult to get the metal alloy 118 to flow into these features using conventional techniques.

As shown in the example implementation 300 of FIG. 3, for instance, a cavity 128 defined by the mold portions 124, 126 may be shaped to form the wall 202 and the features 204, 206. A flow of the metal alloy 118 into the cavity 128 at relatively thin thickness may cause the metal alloy 114 to cool before filling the cavity 128 and thus may be leave voids in the cavity 128 between the metal alloy 114 and surfaces of the cavity 128. These voids may consequently have an adverse effect on the article 114 being molded. Accordingly, techniques may be employed to reduce and even eliminate formation of the voids, an example of which is described in the following discussion and corresponding figure.

FIG. 4 depicts a system 400 in an example implementation in which an injection distribution device 402 is used to physically couple an outflow of the injected metal alloy from the injection device 104 to a mold 120 of the molding device 106. Pressure used to inject the metal alloy 118 to form the article 114 may set to encourage a uniform fill of the cavity 128 of the mold 120.

For example, a pressure may be employed by the injection device 104 that is sufficient to form an alpha layer (e.g., skin) on an outer surface of the metal alloy 118 as it flows through the mold 120. The alpha layer, for instance, may have a higher density at a surface than in the “middle” of the metal alloy 118 when flowing into the mold 120. This may be formed based at least in part using relatively high pressures (such as around 40 mega Pascals) such that the skin is pressed against a surface of the mold 120 thereby reducing formation of voids. Thus, the thicker the alpha layer the less chance of forming voids in the mold 120.

Additionally, an injection distribution device 402 may be configured to encourage this flow from the injection device 104 into the mold 120. The injection device 402 in this example includes a runner 404 and a plurality of sub-runners 406, 408, 410. The sub-runners 406-410 are used to distribute the metal alloy 118 into different portions of the mold 120 to promote a generally uniform application of the metal alloy 118.

However, conventional injection distribution devices were often configured such that a flow of the metal alloy 118 or other material was hindered by the branches of the device. The branches formed by sub-runners of convention devices, for instance, may be sized such as to cause an approximate forty percent flow restriction between a runner and the sub-runners that were configured to receive the metal alloy 118. Thus, this flow restriction could cause cooling of the metal alloy 118 as well as counteract functionality supported through use of particular pressures (e.g., about 40 mega Pascals) used to form alpha layers.

Accordingly, the injection distribution device 402 may be configured such that a decrease in flow of the metal alloy 118 through the device is not experienced. For example, a size of a cross section 412 taken of the runner 404 may be approximated by an overall size of a cross section 414 taken of the plurality of sub-runners 406, 408, 410, which is described further below and shown in relation to a corresponding figure.

FIG. 5 depicts an example implementation 500 showing comparison of respect cross sections 412, 414 of the runner 404 and the plurality of sub-runners 406-410. The cross section 412 of the runner 404 is approximately equal to or less than a cross section 414 overall of the plurality of sub-runners 406-408. This may be performed by varying a diameter (e.g., including height and/or width) such that flow is not reduced as the metal alloy 118 passes through the injection distribution device 104.

For example, the runner 404 may be sized to coincide with an injection port of the injection device 104 and the plurality of sub-runners 406-410 may get progressively shorter and wider to coincide with a form factor of the cavity 128 of the mold 120. Additionally, although a single runner 404 and three sub-runners 406-410 are shown it should be readily apparent that different numbers and combinations are also contemplated without departing from the spirit and scope thereof. Additional techniques may also be employed to reduce a likelihood of voids in the article, another example of which is described as follows.

FIG. 6 depicts a system 600 in an example implementation in which a vacuum device is employed to create negative pressure inside a cavity of the mold 120 to promote flow of the metal alloy 118. As previously described, metal alloys 118 such as one primarily comprised of magnesium may be resistant to flow, especially for thickness that are less than a millimeter. This problem may be exacerbated when confronted with forming an article that is approximately two hundred millimeters long or greater and thus conventional techniques were limited to articles smaller than that.

For example, it may be difficult using conventional techniques to fill a cavity under conventional techniques to form a part of a housing of a computing device that has walls having a thickness of approximately 0.65 millimeters and width and length of greater than 100 millimeters and one hundred and fifty millimeters, respectively (e.g., approximately 190 millimeters by 240 millimeters for a tablet). This is because the metal alloy 118 may cool and harden, especially at those thicknesses and lengths due to the large amount of surface area in comparison with thicker and/or shorter articles. However, the techniques described herein may be employed to form such an article.

In the system 600 of FIG. 6, a vacuum device 602 is employed to bias a flow of the metal alloy 118 through the cavity 128 to form the article 114. For example, the vacuum device 602 may be configured to form negative pressure within the cavity 128 of the mold 120. The negative pressure (e.g., 0.4 bar) may include a partial vacuum formed to remove air from the cavity 218, thereby reducing a chance of formation of air pockets as the cavity 128 is filled with the metal alloy 118.

Further, the vacuum device 602 may be coupled to particular areas of the mold 120 to bias the flow of the metal alloy 118 in desired ways. The article 114, for instance, may include areas that are feature rich (e.g., as opposed to sections having fewer features, the wall 202, and so on) and thus may restrict flow in those areas. Additionally, particular areas might be further away from an injection port (e.g., at the corners that are located closer to the vacuum device 602 than the injection device 104).

In the illustrated instance, the vacuum device 602 is coupled to areas that are opposite areas of the mold 120 that receive the metal alloy 118, e.g., from the injection device 104. In this way, the metal alloy 118 is encouraged to flow through the mold 120 and reduce voids formed within the mold 120 due to incomplete flow, air pockets, and so on. Other techniques may also be employed to bias flow of the metal alloy 118, another example of which is described as follows and shown in an associated figure.

10 FIG. 7 depicts a system 700 in an example implementation in which a mold 120 includes one or more overflows 702, 704 to bias a flow of metal alloy 118 through a mold 120. As previously described, characteristics of the article 114 to be molded may cause complications, such as due to relative 15 thinness (e.g., less than one millimeter), length of article (e.g., 100 millimeters or over), shape of article 114 (e.g., to reach corners on the opposing side of the cavity 128 from the injection device 104), features and feature density, and so on. These complications may make it difficult to get the metal 20 alloy 118 to flow to particular portions of the mold 120, such as due to cooling and so forth.

25 In this example, overflows 702, 704 are utilized to bias flow of the metal alloy 118 towards the overflows 702, 704. The overflows 702, 704, for instance, may bias flow toward the 30 corners of the cavity 128 in the illustrated example. In this way, a portion of the cavity 128 that may be otherwise difficult to fill may be formed using the metal alloy 118 without introducing voids. Other examples are also contemplated, such as to position the overflows 702, 704 based on feature 35 density of corresponding portions of the cavity 128 of the mold 120. Once cooled, material (e.g., the metal alloy 118) disposed within the overflows 702, 704 may be removed to form the article 114, such as by a machining operation.

Thus, the overflows 702, 704 may be utilized to counteract 35 a “cold material” condition in which the material (e.g., the metal alloy 118) does not fill the cavity 128 completely, thus forming voids such as pinholes. The colder material, for 40 instance, may exit the overflows 702, 704 thus promoting contact of hotter material (e.g., metal alloy 118 still in substantially liquid form) to form the article 114. This may also aide a microstructure of the article 114 due to the lack of imperfections as could be encountered otherwise.

45 FIG. 8 depicts an example implementation 800 in which a protrusion is utilized to reduce an effect of thermal expansion 50 caused by varying degrees of thickness of an article 114 to be 55 molded. As previously described, injection molding was traditionally utilized to form plastic parts. Although these techniques were then expanded to metal alloys, conventional techniques were limited to relatively small sizes (e.g., watch parts) due to thermal expansion of the material, which could cause inconsistencies in articles larger than a relatively small size, e.g., watch parts. However, techniques are described herein which may utilize to counteract differences in thermal expansion, e.g., due to differences in thickness of the article, and as such may be used to support manufacture of larger articles, such as articles over 100 millimeters.

The example implementation 800 is illustrated using first and second stages 802, 804. At the first stage 802, the mold 120 is shown as forming a cavity 128 to mold an article. The 60 cavity 128 is configured to have different thicknesses to mold different parts of the article 114, such as a wall 202 and a feature 206. As illustrated, the feature 206 has a thickness that is greater than a thickness of the wall 202. Accordingly, the feature 206 may exhibit a larger amount of contraction than 65 the wall 202 due to thermal expansion of the metal alloy 118. Using conventional techniques, this caused a depression in a side of the article that is opposite to the feature 206. This

depression made formation of a substantially flat surface on a side of the article that opposed the feature 206 difficult if not impossible using conventional injection molding techniques.

Accordingly, the cavity 126 of the mold may be configured to form a protrusion 806 on an opposing side of the feature. The protrusion 806 may be shaped and sized based at least in part on thermal expansion (and subsequent contraction) of the metal alloy 118 used to form the article. The protrusion 806 may be formed in a variety of ways, such as to have a minimum radius of 0.6 mm, use of angles of thirty degrees or less, and so on.

Therefore, once the metal alloy 118 cools and solidifies as shown in the second stage 804, the article 114 may form a substantially flat surface that includes an area proximal to an opposing side of the feature as well as the opposing side of the feature 206, e.g., the wall 202 and an opposing side of the feature 206 adjacent to the wall 202. In this way, the article 114 may be formed to have a substantially flat surface using a mold 120 having a cavity 128 that is not substantially flat at a corresponding portion of the cavity 128 of the mold 120.

FIG. 9 depicts an example implementation 900 in which a mold is employed that includes edges configured to reduce voids. This implementation 900 is also shown using first and second stage 902, 904. As previously described, injection molding was traditionally performed using plastics. However, when employed to mold a metal alloy 118, conventional techniques could be confronted with reduced flow characteristics of the metal alloy 118 in comparison with the plastics, which could cause voids.

Accordingly, techniques may be employed to reduce voids in injection molding using a metal alloy 118. For example, at the first stage 902 molding portions 124, 126 of the mold 120 are configured to form a cavity 128 as before to mold an article 114. However, the cavity 128 is configured to employ radii and angles that promote flowability between the surface of the cavity 218 and the metal alloy 118 to form the article 114 without voids.

For example, the article 114 may be configured to include portions (e.g., a wall) that have a thickness of less than one millimeter, such as approximately 0.65 millimeter. Accordingly, a radius 906 of approximately 0.6 to 1.0 millimeters may be used to form an edge of the article 114. This radius 906 is sufficient to promote flow of a metal alloy 118 comprised primarily of magnesium through the cavity 128 of the mold 120 from the injection device 104 yet still promote contact. Other radii are also contemplated, such as one millimeter, two millimeters, and three millimeters. Additionally, larger radii may be employed with articles having less thickness, such as a radius of approximately twelve millimeters for an article 114 having walls with a thickness of approximately 0.3 millimeters.

In one or more implementations, these radii may be employed to follow a likely direction of flow of the metal alloy 118 through the cavity 128 in the mold 120. A leading and/or trailing edge of a feature aligned perpendicular to the flow of the metal alloy 118, for instance, may employ the radii described above whereas other edges of the feature that run substantially parallel to the flow may employ “sharp” edges that do not employ the radii, e.g., have a radius of less than 0.6 mm for an article 114 having walls with a thickness of approximately 0.65 millimeters.

Additionally, techniques may be employed to remove part of the metal alloy 118 to form a desired feature. The metal alloy 118, for instance, may be shaped using the mold 120 as shown in the first stage 902. At the second stage, edges of the article 114 may be machined to “sharpen” the edges, e.g., stamping, grinding, cutting, and so on. Other examples are

also contemplated as further described in the following discussion of the example procedures.

#### Example Procedures

The following discussion describes injection molding techniques that may be implemented utilizing the previously described systems and devices. Aspects of each of the procedures may be implemented in hardware, firmware, or software, or a combination thereof. The procedures are shown as a set of blocks that specify operations performed by one or more devices and are not necessarily limited to the orders shown for performing the operations by the respective blocks. In portions of the following discussion, reference will be made to FIGS. 1-9.

FIG. 10 depicts a procedure 1000 in an example implementation in which an article is injection molded using a mold that employs overflows. An article is injection molded using a metal alloy comprised primarily of magnesium using a molding device having a plurality of molding portions that form a cavity that defines an article to be molded using the metal alloy and one or more overflows that are positioned to bias flow of the metal alloy toward parts of the cavity that correspond to the overflows (block 1002). As shown in FIG. 7, for instance, the overflows 702, 704 may be positioned to bias flow towards associated regions of the mold 120. The overflows 702, 704 may also be used to remove metal alloy 118 that has cooled during flow through the mold 120 such that subsequent metal alloy that is injected into the mold 120 may remain in a liquid form sufficient to contact the surface of the cavity as opposed to the cooled metal alloy 118 that may cause pin holes and other imperfections.

The metal alloy collected in the one or more overflows is removed from the metal alloy molded using the cavity to form the article (block 1004). This may be performed using a stamping, machining, or other operation in which the metal alloy 118 disposed in the overflows is separated from the metal alloy 118 in the cavity 128 of the mold 120 that is used to form the article 114, e.g., a housing of a hand-held computing device such as a tablet, phone, and so on.

FIG. 11 depicts a procedure 1100 in an example implementation in which a mold is formed that employs overflows. A mold is formed that includes a plurality of molding portions (block 1102). The molding portions may be used to form a cavity that define an article to be molded using a metal alloy (block 1104), such as a metal alloy comprised primarily of magnesium.

One or more flows may also be formed as part of the molding portions that are positioned to bias flow of the metal alloy injected through the cavity toward parts of the cavity that correspond to the overflows (block 1106). As before, these overflows may be positioned due to feature density of the article, difficult locations of the cavity to fill, located to remove “cooled” metal alloy, and so on.

FIG. 12 depicts a procedure 1200 in an example implementation in which a protrusion is formed to at least partially counteract thermal expansion of the metal alloy and subsequent contraction caused by cooling of the metal alloy. A metal alloy is injected into a mold having a plurality of molding portions that define a cavity that corresponds to an article to be molded. The mold defines a portion of the cavity that defines a feature for the article having a thickness that is greater than a thickness of an area of the article defined by the cavity that is proximal to the feature. The mold also defines a protrusion for the article aligned as substantially opposing the feature, the protrusion being sized such that upon solidifying of the metal alloy that forms the article, the protrusion reduces an effect of thermal expansion on a portion of the article that is aligned as substantially opposing the feature (block 1202).

The protrusion, for instance, may be formed as an indentation in part of the cavity 128 of the mold 120.

The metal alloy is removed from the cavity of the mold after solidifying of the metal alloy within the mold (block 1204). As stated above, the protrusion may be used to offset an effect of thermal expansion and subsequent contraction of the metal alloy 118, such as to form a substantially flat surface on a side of the article opposite to the feature.

FIG. 13 depicts a procedure 1300 in an example implementation in which a mold is formed that is configured to form a protrusion on an article to counteract an effect of thermal expansion. A mold is formed having a plurality of molding portions to form an article using a metal alloy that is defined in the mold using a cavity (block 1302). This may include forming a portion of the cavity that defines a feature for the article having a thickness that is greater than a thickness of an area of the article defined by the cavity that is proximal to the feature (block 1304).

The mold may also be configured to form a protrusion for the article aligned on a side of the cavity that is opposite to a side including the feature, the protrusion being sized as being proportional to the thickness of the feature such that upon solidifying of the metal alloy that forms the article, the protrusion reduces an effect of thermal expansion on the side of the article that is opposite to the feature (block 1306). In this way, subsequent cooling of the metal alloy and corresponding contraction may be addressed to reduce the effect of the thermal expansion on the article.

FIG. 14 depicts a procedure 1400 in an example implementation in which a radius is employed to limit formation of voids of the article. A metal alloy is injected into a mold having a plurality of molding portions that define a cavity that corresponds to an article to be molded including walls with a thickness of less than one millimeter with one or more features disposed thereon having edges with a radius of at least 0.6 millimeter (block 1402). As previously described, metal alloys may introduce complications not encountered using plastics, such as quicker cooling and resistance to flow through a mold 120, especially for articles having a thickness of under one millimeter. Accordingly, the radius may be employed to reduce voids caused by sharp edges.

At least a portion of the radius of the edge is machined to define the feature of the article after removal of the metal alloy from the cavity (block 1404). In this way, a sharp edge may be provided on the device yet a likelihood of voids reduced. A variety of other examples are also contemplated as previously described in relation to FIG. 9.

## CONCLUSION

Although the invention has been described in language specific to structural features and/or methodological acts, it is to be understood that the invention defined in the appended claims is not necessarily limited to the specific features or acts described. Rather, the specific features and acts are disclosed as example forms of implementing the claimed invention.

What is claimed is:

1. A method comprising:  
injecting a metal alloy into a mold having a plurality of molding portions that define a cavity that corresponds to an article to be molded, the mold defining:

a portion of the cavity that defines a feature for the article having a thickness that is greater than a thickness of an area of the article defined by the cavity that is proximal to the feature; and

a protrusion for the article aligned as substantially opposing the feature, the protrusion being sized such that upon solidifying of the metal alloy that forms the article, the protrusion reduces an effect of thermal expansion on a portion of the article that is aligned as substantially opposing the feature; and

removing the metal alloy from the cavity of the mold after solidifying of the metal alloy within the mold.

2. A method as described in claim 1, wherein the protrusion is sized as proportional to the thickness of the feature and a coefficient of thermal expansion of the metal alloy.

3. A method as described in claim 1, wherein the protrusion reduces the effect of thermal expansion on the portion of the article that is aligned as substantially opposing the feature such that an area proximal to the portion and the portion form a substantially flat surface after the solidifying of the metal alloy.

4. A method as described in claim 1, wherein the metal alloy is comprised primarily of magnesium.

5. A method as described in claim 1, wherein the thickness of the area proximal to the feature is less than one millimeter and the thickness of the protrusion is greater than one millimeter.

6. A method as described in claim 5, wherein the thickness of the area is approximately 0.65 millimeter.

7. A method comprising:

forming a mold comprising a plurality of molding portions to form an article using a metal alloy that is defined in the mold using a cavity, the forming including:

forming a portion of the cavity that defines a feature for the article having a thickness that is greater than a thickness of an area of the article defined by the cavity that is proximal to the feature; and

forming a protrusion for the article aligned on a side of the cavity that is opposite to a side including the feature, the protrusion being sized as being proportional to the thickness of the feature such that upon solidifying of the metal alloy that forms the article, the protrusion reduces an effect of thermal expansion on the side of the article that is opposite to the feature.

8. A method as described in claim 7, wherein the protrusion is sized based also on a coefficient of thermal expansion of the metal alloy.

9. A method as described in claim 7, wherein the protrusion is sized to form a substantially flat surface after the solidifying of the metal alloy.

10. A method as described in claim 7, wherein the protrusion is defined in the cavity such that a corresponding surface of the cavity that corresponds to the protrusion is not flat.

11. A method as described in claim 7, wherein the metal alloy is comprised primarily of magnesium.

12. A method as described in claim 7, wherein the thickness of the area proximal to the feature is less than one millimeter and the thickness of the protrusion is greater than one millimeter.